

Patented Mar. 7, 1933

1,900,850

# UNITED STATES PATENT OFFICE

MAHLIN S. HANSEN, OF INDIANAPOLIS, INDIANA, ASSIGNOR TO PETER C. REILLY, OF INDIANAPOLIS, INDIANA

## FROTH-FLOTATION PROCESS FOR SLIME-CONTAINING ORE PULPS

No Drawing.

Application filed July 31, 1931. Serial No. 554,385.

This invention relates to improvements in the concentration of "oxidized ores" by the froth-flotation process, and has special reference to a means for overcoming the detrimental effect of slimes in the separation of minerals by the froth-flotation process.

This invention is based on the discovery that the use of fluosilicates of the class including hydrofluosilicic acid ( $H_2SiF_6$ ), sodium fluosilicate ( $Na_2SiF_6$ ), potassium fluosilicate ( $K_2SiF_6$ ), calcium fluosilicate ( $CaSiF_6$ ), magnesium fluosilicate ( $MgSiF_6$ ), and ammonium fluosilicate ( $(NH_4)_2SiF_6$ ), in the froth-flo-  
10 tation operation, modifies the character of "oxi-  
15 dized-ore" pulps so that a sharper, cleaner, and more satisfactory flotation can be accom-  
plished. In some cases the use of these com-  
pounds makes it possible to apply the flo-  
tation process where it would otherwise com-  
20 mercially fail.

As is well known, the froth-flotation proc-  
ess necessitates the grinding of an ore to a  
suitable fineness and in doing this a part  
of the ore is reduced to a size commonly  
25 known as slimes. Also, many ores contain  
a relatively large amount of slimes in their  
natural state; particularly ores commonly  
known to miners and millmen as "oxidized  
ores", which may be partly or wholly true  
30 carbonates, but are often partly or largely  
sulfates, hydroxides, oxides, and analogous  
compounds, and are usually quite complex.  
These slimes usually contain a relatively large  
amount of colloidal slimes, both organic and  
35 inorganic, and quasi-colloidal slimes. In  
general the natural slimes contain more of the  
colloidal and quasi-colloidal matter than do  
slimes produced artificially by grinding.

With most ores the presence of slimes in  
40 the pulp is a serious impediment to the suc-  
cessful concentration of the mineral values  
by the froth-flotation process, and in many  
cases the concentration of mineral is made  
impossible by the presence of slimes.

45 The actual cause of the deleterious effect

of slimes in the froth-flotation process has not  
been entirely and satisfactorily explained.  
Apparently several effects are present. The  
slimes may absorb or adsorb, or otherwise  
50 tend to render ineffective, the frothing and  
collecting agents which are used. The slimes  
may armor the froth-bubble so completely as  
to exclude from the froth the mineral par-  
ticles of larger size. Also, it has been shown  
55 by recent workers that slimes adhere to the  
surfaces of mineral particles, thereby caus-  
ing the mineral particles to resist flotation in  
a manner similar to that of gangue particles.

I have discovered that by the use of small  
amounts of fluosilicates of the class includ-  
ing hydrofluosilicic acid ( $H_2SiF_6$ ), sodium  
fluosilicate ( $Na_2SiF_6$ ), potassium fluosilicate  
( $K_2SiF_6$ ), and ammonium fluosilicate  
( $(NH_4)_2SiF_6$ ), and in some cases calcium fluo-  
silicate ( $CaSiF_6$ ) and magnesium fluosilicate  
( $MgSiF_6$ ), in the froth-flotation of "oxi-  
60 dized ores", the slimes are dispersed and their  
deleterious effects are overcome and the fol-  
lowing advantages are obtained in the froth-  
fotation process:

(1) A sharper, cleaner, and more satisfac-  
tory concentration of mineral in "oxidized-  
ore" pulps containing slimes.

(2) A ready concentration of mineral in  
slime-containing "oxidized ore" pulps which  
are in general difficult to concentrate by the  
froth-flotation process.

(3) A concentration of mineral in cer-  
tain mineral "oxidized-ore" pulps consist-  
ing entirely of slimes.

(4) A higher grade concentrate.

(5) A lower loss in the tailing.

(6) Generally, the ability to use a smaller  
amount of other necessary flotation reagents.

(7) Generally, a more rapid formation of  
the froth.

(8) A froth which is highly selective in its  
action.

Examples of the use of these fluosilicates  
are given below: Example I shows the use

- of hydrofluosilicic acid and of sodium fluosilicate respectively on an "oxidized-ore" pulp containing both sands and slimes, both in a neutral circuit and in an alkaline circuit. Example II shows the use of these compounds on an "oxidized-ore" pulp substantially free from slimes. Example III shows the use of the same materials on an "oxidized ore" pulp containing slimes only.
- 10 In these examples, the flotation reagent and the selectors named are given merely by way of example, as any suitable flotation reagent and any suitable selector may be used.

15 *Example I*

- A so-called "oxidized ore" of copper, containing some sulfid minerals and other minerals such as atacamite ( $\text{CuCl}_2 \cdot 3\text{Cu}(\text{OH})_2$ ), brochantite ( $\text{CuSO}_4 \cdot 3\text{Cu}(\text{OH})_2$ ), and chalcanthite ( $\text{CuSO}_4 \cdot 5\text{H}_2\text{O}$ ), washed free of soluble salts but not deslimed, and containing 1.06% copper, was floated, using 0.15 lb. pine oil per ton of ore, in conjunction with other reagents as indicated below in pounds per ton of ore.

| Test | Selector | $\text{H}_2\text{SiF}_6$ hydro-fluosilicic acid | $\text{Na}_2\text{SiF}_6$ sodium fluosilicate | $\text{Ca}(\text{OH})_2$ | % copper recovery  |
|------|----------|-------------------------------------------------|-----------------------------------------------|--------------------------|--------------------|
| 30   |          |                                                 |                                               |                          |                    |
| a    | 0.25 lb. | Potassium ethyl xanthate.                       | None.                                         | None.                    | 2.0 lbs. 28.0      |
| b    | 0.25 lb. | Potassium ethyl xanthate.                       | None.                                         | 2.0 lbs.                 | 2.0 lbs. 49.0      |
| c    | 0.25 lb. | Potassium ethyl xanthate.                       | 1.0 lb.                                       | None.                    | 2.0 lbs. 45.0      |
| 35   | d        | 0.15 lb.                                        | Dithiocyan-o-leic acid.                       | None.                    | None. No recovery. |
| e    | 0.15 lb. | Dithiocyan-o-leic acid.                         | None.                                         | 4.0 lbs.                 | None. 86.0         |
| f    | 0.15 lb. | Dithiocyan-o-leic acid.                         | 1.0 lb.                                       | None.                    | None. 84.0         |

- 40 (The use of dithiocyan-o-leic acid as a selector is the subject-matter of my co-pending application Serial No. 522,790, filed March 14, 1931.)

45 *Example II*

- Some of the same "oxidized ore" as used in Example I was washed free from soluble salts, and then ground to flotation size; and the ore pulp was separated into two parts containing the sands and slimes respectively. The sands were used in tests given under this example; while the slimes were used in tests given under Example III. In the following tests of this Example II, 0.15 lb. of pine oil was used per ton of ore for the frothing agent, in conjunction with other reagents used in pounds per ton of ore as indicated below.

| Test | Selector                        | Hydro fluosilicic acid | Sodium fluosilicic acid | % Copper recovery |
|------|---------------------------------|------------------------|-------------------------|-------------------|
| 60   |                                 |                        |                         |                   |
| g    | 0.15 lb. Dithiocyan-o-leic acid | None.                  | None.                   | 61.0              |
| h    | 0.15 lb. Dithiocyan-o-leic acid | None.                  | 1.0 lb.                 | 99.0              |
| i    | 0.15 lb. Dithiocyan-o-leic acid | 1.0 lb.                | None.                   | 92.0              |

*Example III*

The following tests were made on the slimes which were separated from the sands used in Example II. In these tests 0.20 lb. 70 of pine oil per ton of the "oxidized ore" was used as the frothing agent, in conjunction with other reagents in pounds per ton of ore as indicated below.

| Test | Selector                       | Hydro fluosilicic acid | Sodium fluosilicic acid | % Copper recovery |
|------|--------------------------------|------------------------|-------------------------|-------------------|
| f    | .25 lb. Dithiocyan-o-leic acid | None.                  | None.                   | None.             |
| k    | .25 lb. Dithiocyan-o-leic acid | None.                  | 6.0 lbs.                | 88.0              |
| l    | .25 lb. Dithiocyan-o-leic acid | 2.0 lbs.               | None.                   | 84.0              |

These examples show very markedly the beneficial effect that the use of these fluosilicates as dispersing agents for the slimes has 85 on the copper recovery.

Following similar procedures as those described in the above examples, but using another type of "oxidized ore" in which the valuable constituents were vanadium minerals, I have used calcium fluosilicate and ammonium fluosilicate, respectively, and have obtained a high recovery of the vanadium minerals in the form of a high-grade 90 product.

Although I have given specific examples to illustrate my invention, they are illustrative only. Variations in the quantities of reagents employed, the combinations of reagents, the kind of "oxidized ore," and the 95 steps of the procedure, may be varied in practice as determined by the composition of the given "oxidized ore" without departing from the invention claimed.

I have found that the fluosilicates can be 105 used in the crude form as well as in the relatively pure form. I have used with excellent results the crude hydrofluosilicic acid and sodium fluosilicate which are produced as by-products in the manufacture of fertilizer from phosphate rock. Likewise, I have used the crude form of calcium fluosilicate with satisfactory results, as well as the relatively pure product.

These fluosilicates can be used with desirable and effective results in alkaline, neutral, or acid circuits. In some cases, as with calcium fluosilicate, the action is better in 110 neutral or acid circuits.

I claim as my invention:

1. The process of concentrating slime-containing "oxidized ore" pulps by froth flotation, comprising modifying a slime-containing "oxidized-ore" pulp with a fluosilicate of the class including hydrofluosilicic acid, 125 sodium fluosilicate, potassium fluosilicate, calcium fluosilicate, magnesium fluosilicate, and ammonium fluosilicate; and subjecting the modified "oxidized-ore" pulp to the froth-flotation process.

2. The process of concentrating slime-containing "oxidized-ore" pulps by froth flotation, comprising modifying a slime-containing "oxidized-ore" pulp with a fluosilicate of the class including hydrofluosilicic acid, sodium fluosilicate, potassium fluosilicate, calcium fluosilicate, magnesium fluosilicate, and ammonium fluosilicate.

10 the froth-flotation process with pine oil as the frothing reagent.

3. The process of concentrating slime-containing "oxidized-ore" pulps by froth flotation, comprising modifying a slime-containing "oxidized-ore" pulp with hydrofluosilicic acid; and subjecting the modified "oxidized-ore" pulp to the froth-flotation process.

4. The process of concentrating slime-containing "oxidized-ore" pulps by froth flotation, comprising modifying a slime-containing "oxidized-ore" pulp with sodium fluosilicate; and subjecting the modified "oxidized-ore" pulp to the froth-flotation process.

25 5. The process of concentrating slime-containing "oxidized-ore" pulps by froth flotation, comprising modifying a slime-containing "oxidized-ore" pulp with ammonium fluosilicate; and subjecting the modified "oxidized-ore" pulp to the froth-flotation process.

35 6. The process of concentrating slime-containing pulps of "oxidized ores" by froth flotation, comprising modifying the slime-containing pulp of an "oxidized ore" with a fluosilicate of the class including hydrofluosilicic acid, sodium fluosilicate, potassium fluosilicate, calcium fluosilicate, magnesium fluosilicate, and ammonium fluosilicate; and subjecting the modified "oxidized-ore" pulp to the froth-flotation process.

45 7. The process of concentrating slime-containing pulps of copper-bearing "oxidized ores" by froth flotation, comprising modifying the slime-containing pulp of a copper-bearing "oxidized ore" with a fluosilicate of the class including hydrofluosilicic acid, sodium fluosilicate, potassium fluosilicate, calcium fluosilicate, magnesium fluosilicate, and ammonium fluosilicate; and subjecting the modified "oxidized-ore" pulp to the froth-flotation process.

55 8. In the froth-flotation process for concentrating minerals of "oxidized ores", the modification of an "oxidized-ore" pulp to which the process is applied by the introduction as a dispersing agent of a fluosilicate of the class including hydrofluosilicic acid, sodium fluosilicate, potassium fluosilicate, calcium fluosilicate, magnesium fluosilicate, and ammonium fluosilicate.

60 9. The step in the process of concentrating an "oxidized-ore" pulp by froth flotation, comprising dispersing slimes present in an "oxidized-ore" pulp by the addition to said

pulp of a fluosilicate of the class including hydrofluosilicic acid, sodium fluosilicate, potassium fluosilicate, calcium fluosilicate, magnesium fluosilicate, and ammonium fluosilicate.

70 In witness whereof, I have hereunto set my hand at Indianapolis, Indiana, this 29th day of July, A. D. one thousand nine hundred and thirty-one.

MAHLIN S. HANSEN. 75

80

85

90

95

100

105

110

115

120

125

130

**Certificate of Correction**

Patent No. 1,900,850.

March 7, 1933.

**MAHLIN S. HANSEN**

It is hereby certified that error appears in the printed specification of the above-numbered patent requiring correction as follows: Page 1, line 75, page 2, line 9, and line 122, claim 1, for "oxidized ore" read "*oxidized-ore*"; page 2, after line 25, in the boxed heading to table, column 6, for "Ca-(OH)<sub>2</sub>" read *Ca(OH)<sub>2</sub>*; page 3, line 37, claim 6, after the syllable "silicic" strike out the comma; and that the said Letters Patent should be read with these corrections therein that the same may conform to the record of the case in the Patent Office.

Signed and sealed this 18th day of April, A. D. 1933.

[small]

**M. J. MOORE,**  
*Acting Commissioner of Patents.*